



US006103355A

# United States Patent [19]

Mehta

[11] Patent Number: 6,103,355

[45] Date of Patent: Aug. 15, 2000

[54] **CELLULOSE SUBSTRATES WITH TRANSPARENTIZED AREA AND METHOD OF MAKING SAME**

[75] Inventor: **Rajendra Mehta**, Dayton, Ohio

[73] Assignee: **The Standard Register Company**, Dayton, Ohio

[21] Appl. No.: **09/104,573**

[22] Filed: **Jun. 25, 1998**

[51] Int. Cl.<sup>7</sup> ..... **B32B 3/00**

[52] U.S. Cl. ..... **428/211; 427/164; 427/256; 427/386; 427/391**

[58] **Field of Search** ..... 428/172, 195, 428/211, 537.5; 503/200, 206, 226; 427/164, 256, 386, 391

## [56] References Cited

### U.S. PATENT DOCUMENTS

|           |         |                 |   |
|-----------|---------|-----------------|---|
| 2,760,863 | 8/1956  | Plambeck, Jr.   | . |
| 3,043,805 | 7/1962  | Burg.           | . |
| 3,261,686 | 7/1966  | Celeste et al.  | . |
| 3,380,831 | 4/1968  | Cohen et al.    | . |
| 3,469,982 | 9/1969  | Celeste.        | . |
| 3,661,576 | 5/1972  | Crary.          | . |
| 3,813,261 | 5/1974  | Muller.         | . |
| 3,936,577 | 2/1976  | Watt.           | . |
| 4,128,437 | 12/1978 | Ura et al.      | . |
| 4,198,465 | 4/1980  | Moore et al.    | . |
| 4,237,185 | 12/1980 | Lombardi et al. | . |
| 4,271,227 | 6/1981  | Muller et al.   | . |
| 4,279,717 | 7/1981  | Eckberg et al.  | . |
| 4,319,009 | 3/1982  | Friedli et al.  | . |

|           |         |                     |
|-----------|---------|---------------------|
| 4,362,848 | 12/1982 | Friedli et al. .    |
| 4,416,950 | 11/1983 | Muller et al. .     |
| 4,513,056 | 4/1985  | Vernois et al. .    |
| 4,526,803 | 7/1985  | White.              |
| 4,569,888 | 2/1986  | Muller et al. .     |
| 4,729,506 | 3/1988  | Neubauer.           |
| 4,761,435 | 8/1988  | Murphy et al. .     |
| 4,814,043 | 3/1989  | Rausing et al. .    |
| 5,055,354 | 10/1991 | Simcocke.           |
| 5,207,871 | 5/1993  | Murphy et al. .     |
| 5,232,812 | 8/1993  | Morrison et al. .   |
| 5,416,126 | 5/1995  | Murphy et al. .     |
| 5,418,205 | 5/1995  | Mehta et al. .      |
| 5,663,264 | 9/1997  | Kawai et al. .      |
| 5,732,477 | 3/1998  | Toyama ..... 34/275 |

### FOREIGN PATENT DOCUMENTS

06280198 10/1994 Japan .

Primary Examiner—Bruce H. Hess

Assistant Examiner—Michael Grendzynski

Attorney, Agent, or Firm—Killworth, Gottman, Hagan & Schaeff LLP

## [57] ABSTRACT

A cellulosic substrate which is suitable for use as a mailer or envelope and which has at least one transparentized portion is provided. A method of transparentizing a cellulosic substrate by the application of a transparentizing material which provides enhanced toner adhesion properties, fast penetration rates and which is rapidly and completely cured by exposure to radiation is also provided. Further, these transparentizing materials may be applied without the need for solvents. These features thus permit continuous, in-line transparentization.

32 Claims, 2 Drawing Sheets





FIG. 1



FIG. 2



FIG. 3



FIG. 4



FIG. 5



FIG. 6

**CELLULOSE SUBSTRATES WITH  
TRANSPARENTIZED AREA AND METHOD  
OF MAKING SAME**

**FIELD OF THE INVENTION**

The present invention relates to a cellulosic substrate, and method of making it, suitable for use as an envelope or mailer, and more particularly, to one having at least one transparentized portion.

**BACKGROUND OF THE INVENTION**

As is known, various types of envelopes or mailers with transparent windows exist where the window consists of a cut-out opening in the mailer substrate which is covered by a transparent patch. The transparent patch is usually secured over the cut-out opening by means of an adhesive, and may consist of any suitable film of transparent material such as glassine, cellophane, or polymeric materials including polyester, polyethylene, polycarbonate, polystyrene, and polyethylene terephthalate. The adhesive is generally applied to the mailer substrate around the perimeter of the cut-out opening to join the outer perimeter of the transparent patch thereto. The transparent patch can be secured to either the inside or outside surface of the mailer substrate.

In some modern mailing systems, a mailer is formed from a single sheet after it has been imaged by a non-impact printer. These sheets are stacked in an input hopper and fed as single plies through the printer, after which the sheets are folded to form a mailer. A window is provided to permit the name and address to show through. Added thickness caused by such window patches over die-cut window openings causes mis-shapen stacks and prevents trouble-free feeding.

The typical arrangement of such patches is disadvantageous as the transparent patch is layered on top of or below the substrate making the thickness of the window portion of the sheet greater than that of the remainder of the sheet. As a consequence, such sheets form unstable and uneven stacks, and thus limit the maximum height to which they can be stacked. This stack-height limitation is burdensome to large scale printing operations.

Another disadvantage with mailers having a cut-out opening covered by a transparent patch is that the edges of the transparent patch often get caught by process machinery, such as sheet transport mechanisms in printers. This results in the destruction of the mailer and usually requires the machinery to be stopped so that the destroyed mailer can be removed. Moreover, when heat is employed in such process machinery, the adhesive holding the transparent patch to the mailer substrate can soften, causing the patch to become detached from the mailer substrate.

One alternative to the cut-out/transparent patch type of arrangement is to apply a transparentizing material to a predetermined portion of the cellulosic mailer substrate to thereby form a window. See, for example, U.S. Pat. No. 5,418,205 to Mehta. Such a method entails the impregnation of the cellulosic mailer substrate with transparentizing material. The spaces between the fibers of the substrate are filled by the transparentizing material. In order to make the impregnated portion transparent, the transparentizing material must have a refractive index close to that of cellulose (1.5).

In order to produce high quality cellulosic mailers on a large, industrial scale by employing a transparentizing material, it is desirable that the transparentizing material be capable of achieving at least three important functions:

- 1) the ability to produce a transparentized portion which possesses a number of physical and chemical properties;
- 2) the ability to be converted quickly from a penetrating liquid to a solid after impregnation has occurred; and
- 3) the ability to quickly penetrate the cellulosic mailer substrate in order to fully impregnate the substrate in the shortest time possible.

The drawback to producing mailers in this manner, however, is that most transparentizing materials can perform, at most, only one of the aforementioned functions.

Physically, the transparentized portion of a cellulosic mailer substrate should be physically strong and flexible (i.e., not brittle) and be receptive to inks. Chemically, the transparentized portion should meet U.S. Postal Service 15 specifications for reflectance (sufficient transparency to read the printing beneath the transparentized portion) and PCR ("Print Contrast Ratio"—sufficient contrast between the printing and background beneath the transparentized portion) and should have sufficient resistance to migration and/or volatilization of the transparentizing material from the place where applied on the mailer substrate such that it does not lose its transparency over time.

Conventional transparentizing materials are not capable of producing transparentized window portions which possess all of the aforementioned physical and chemical properties. U.S. Pat. No. 5,076,489 to Steidinger, for example, discloses using either wax or oil as the transparentizing material. Wax produces a brittle transparentized area which is easily marred by physical contact therewith to cause a loss 25 of transparency. In addition, wax is not receptive to inks and therefore cannot be printed upon. Oil tends to migrate and/or volatilize easily, thus resulting in a loss of transparency over time.

In an attempt to overcome these problems, certain liquid 35 polymerizable transparentizing compositions have been utilized. When utilizing polymerizable transparentizing compositions, the paper substrate is first rendered transparent by impregnating it with the liquid polymerizable transparentizing composition. The liquid polymerizable transparentizing composition is then cured *in situ* to solidify the transparentized portion. These polymerizable transparentizing compositions offer several advantages over conventional transparentizing materials, such as wax and oil, in that the end-product is usually strong and flexible and does not lose 40 its transparency over time due to migration or/or volatilization. However, there are problems associated with the use of these polymerizable transparentizing compositions. For example, the rate at which some of the liquid polymerizable transparentizing compositions penetrate a cellulosic substrate 45 is so slow that, after applying the transparentizing composition to the substrate, the substrate must be wound up in a tight roll for a period of time to allow the material to impregnate the substrate. See for example, U.S. Pat. No. 4,416,950 to Muller et al. Such materials are not conducive 50 to the high-speed production of mailers having transparentized windows. In an attempt to overcome the slow rate of penetration associated with known polymerizable transparentizing compositions, solvents have been included with the polymerizable transparentizing composition to lower the 55 viscosity thereof and thereby speed the rate of penetration of the transparentizing composition into the cellulosic mailer substrate (see, e.g., U.S. Pat. No. 4,513,056 to Vernois et al). However, the use of solvents with transparentizing materials 60 is undesirable due to the added process machinery required to evaporate the solvent from the substrate surface and to recover the evaporated solvent. It is also known to include 65 water or water-alcohol mixtures with the transparentizing

material to increase their wetting capabilities and thus increase the rate of penetration into a cellulosic substrate. See, for example, U.S. Pat. No. 3,813,261 to Muller et al. However, the use of water with transparentizing material is typically not considered conducive to high-speed production due to the time associated with removing the water from the cellulosic substrate surface. In addition, most transparentizing agents are non-polar and are not soluble in water. Therefore, they form emulsions which are not suitable for uniform distribution of the transparentizing material onto the cellulosic substrate.

In addition, since most polymerizable transparentizing agents are non polar, they exhibit limited toner adhesion properties, making it difficult to use high speed laser printers to image the transparentized areas on the mailers. This limits the amount of transparentizing material which can be loaded onto the cellulosic substrate and therefore, limits the degree of transparency in the final transparentized cellulosic product.

Further, although many of these polymerizable transparentizing compositions are thermally cured, radiation curing is preferable for reasons of both accuracy and economy. Radiation-curable, solventless liquid paper transparentizing compositions are known, but suffer from one or more of the above-mentioned problems. For example, U.S. Pat. No. 5,418,205 discloses a solventless liquid transparentizing material which quickly penetrates the cellulosic substrate and results in a high quality transparentized portion which is strong and flexible and which does not lose transparency over time. However, the transparentizing material is non-polar. Therefore, it is insoluble in water and its wetting capabilities cannot be increased by the addition of water due to the formation of emulsions. In addition, since the transparentizing material is non-polar, it exhibits limited toner adhesion properties. Therefore, the degree of transparency in the final product is limited.

In addition, many polymerizable transparentizing compositions suffer from incomplete and/or slow crosslinking reactions. Incomplete cross-linking results in a product in which unreacted monomer or oligomer remains in the cured transparentized layer. Unreacted monomer or oligomer in the cured transparentized layer may result in tackiness. Uncured or partially cured transparentized layers which are tacky present various problems, such as blocking (i.e., when two or more forms or transparentized window areas join together and result in problematic printer feeding) and material transfer of uncured constituents to fuser rollers. In addition, unreacted monomer or oligomer in the cured transparentized layer may result in degradation of opacity of the transparentized area.

Other problems associated with polymerizable, 100% solids transparentizing compositions are odor and skin irritation on contact.

Accordingly, it is seen that a need exists in the art for a substrate suitable for use as a mailer or envelope having at least one transparentized portion which can be placed in tall, stable stacks and which does not have equipment-catching edges around the window area. Further, the transparentized portion should be capable of being produced at a rate of speed conducive to high-speed production of mailers without the need for solvents or water. In addition, the liquid polymerizable transparentizing compositions should exhibit good toner adhesion properties. Also, they should be amenable to curing by radiation rather than by thermal polymerization and such radiation curing should occur both rapidly and completely. In addition, such liquid polymerizable transparentizing compositions should exhibit minimal odor and skin-irritating qualities.

#### SUMMARY OF THE INVENTION

Those needs are met by the present invention. Thus, the present invention provides a cellulosic substrate, and method of making it, which has at least one transparentized portion and preferably, wherein a smooth interface exists between the transparentized portion and the remainder of the substrate. In addition, the transparentized portion preferably has a thickness which is no greater than the thickness of the remainder of the substrate. Thus, no machine-catching edges are present, and mailers made from the substrate will form tall, stable stacks due to the ability to form transparent windows without adding thickness to the substrate. Moreover, the present invention also provides a solventless transparentizing material which penetrates the mailer substrate very quickly and completely, and forms a cured polymeric transparentized portion which not only possesses the aforementioned physical and chemical properties, but also exhibits an improved degree of transparency. In this manner, a very high-quality transparentized portion can be formed on cellulosic mailer substrates in a fast, continuous, in-line process, without the need for recovering a solvent. Further the present invention provides a liquid polymerizable transparentizing compositions which exhibits good toner adhesion properties and is cured by radiation rather than by thermal polymerization and which cure both rapidly and completely. In addition, the liquid polymerizable transparentizing compositions of the present invention exhibit minimal odor and skin-irritating qualities.

The present invention provides a cellulosic substrate suitable for use as an envelope or mailer. The cellulosic substrate has at least one transparentized portion which comprises an area on the substrate which has been impregnated with a polymerized transparentizing material. In certain embodiments, the transparentized portion is thinner than the remainder of the substrate. Preferably, the transparentized portion has a smooth interface between itself and the remainder of the substrate, and the transparentized portion has a thickness which is no greater than the thickness of the remainder of the substrate. "Smooth interface" means one in which no loose or sharp edges are present which could get caught in process equipment and cause jams or tears. "Transparentized" means that there is sufficient transparency to read printing beneath the transparentized portion of the substrate (reflectance of at least 50% in the red spectrum and at least 45% in the green spectrum), and sufficient contrast between the printing and background portion beneath the transparentized portion to provide a print contrast ratio of at least 30%.

The radiation curable transparentizing composition of the present invention comprises a free-radical catalyzable constituent; a cationic catalyzable constituent; and a catalyst. As used herein, the term "cationic catalyzable constituent" refers to a vinyl ether, a polyepoxide, a mixture of vinyl ethers, a mixture of polyepoxides, or a mixture of at least one of a vinyl ether and at least one of a polyepoxide. As used herein, the term "free radical catalyzable constituent" refers to compounds or Formula I or mixtures of compounds of Formula I:



wherein

R'' is any mono- or polyfunctional organic radical;

R is H or  $\text{CH}_3$ ;  
 R' is H or  $-\text{C}(\text{O})\text{C}(\text{R})=\text{CH}_2$ , with the proviso that  $-\text{C}(\text{O})\text{C}(\text{R})=\text{CH}_2$  occurs at least once;  
 x is an integer 0-4 and indicates the number of functional groups on R" which are reactive with ethylene or propylene oxide;  
 z is an integer 1-4 and may vary independently of x and n;  
 n is an integer 0-20 and is independent of x and z; and  
 wherein if any of R, R', or R" are greater than one, their identities and the number of each may be the same or different. As used herein, the term "catalyst" refers to a photocatalyst selected from a free radical catalyst, a mixture of free radical catalysts, a living cationic catalyst, a mixture of living cationic catalysts, or mixtures of at least one of a free radical catalyst and at least one of a living cationic catalyst.

Thus, in one embodiment, there is provided a method of transparentizing a cellulosic substrate which comprises the steps of a) providing a cellulosic substrate; b) applying to at least one surface of the substrate a transparentizing composition comprising: 1) at least one of a polyepoxide; 2) and at least one of a compound or mixture of compounds of Formula I; and 3) at least one of a free radical catalyst; and c) curing the transparentizing composition with radiation.

In another embodiment, there is provided a method of transparentizing a cellulosic substrate which comprises the steps of: a) providing a cellulosic substrate; b) applying to at least one surface of the substrate a transparentizing composition comprising: 1) at least one of a vinyl ether in admixture with at least one of a polyepoxide; 2) at least one of a compound of Formula I; and 3) at least one of a free radical catalyst; and c) curing the transparentizing composition with radiation.

In another embodiment, there is provided a method of transparentizing a cellulosic substrate which comprises the steps of: a) providing a cellulosic substrate; b) applying to at least one surface of the substrate a transparentizing composition comprising: 1) at least one of a polyepoxide; 2) at least one of a compound of Formula I; and 3) at least one of a living cationic catalyst; and c) curing the transparentizing composition with radiation.

In another embodiment, there is provided a method of transparentizing a cellulosic substrate which comprises the steps of: a) providing a cellulosic substrate; b) applying to at least one surface of the substrate a transparentizing composition comprising: 1) at least one of a vinyl ether; 2) at least one of a compound of Formula I; and 3) at least one of a living cationic catalyst; and c) curing the transparentizing composition with radiation.

In another embodiment, there is provided a method of transparentizing a cellulosic substrate which comprises the steps of: a) providing a cellulosic substrate; b) applying to at least one surface of the substrate a transparentizing composition comprising: 1) at least one of a vinyl ether in admixture with at least one of a polyepoxide; 2) at least one of a compound of Formula I; and 3) at least one of a living cationic catalyst; and c) curing the transparentizing composition with radiation.

In another embodiment, there is provided a method of transparentizing a cellulosic substrate which comprises the steps of: a) providing a cellulosic substrate; b) applying to at least one surface of the substrate a transparentizing composition comprising: 1) at least one of a polyepoxide; 2) at least one of a compound of Formula I; and 3) at least one of a free radical catalyst in admixture with at least one of a living cationic catalyst; and c) curing the transparentizing composition with radiation.

In another embodiment, there is provided a method of transparentizing a cellulosic substrate which comprises the steps of: a) providing a cellulosic substrate; b) applying to at least one surface of the substrate a transparentizing composition comprising: 1) at least one of a vinyl ether; 2) at least one of a compound of Formula I; and 3) at least one of a free radical catalyst in admixture with at least one of a living cationic catalyst; and c) curing the transparentizing composition with radiation.

In another embodiment, there is provided a method of transparentizing a cellulosic substrate which comprises the steps of: a) providing a cellulosic substrate; b) applying to at least one surface of the substrate a transparentizing composition comprising: 1) at least one of a vinyl ether in admixture with at least one of a polyepoxide; 2) at least one of a compound of Formula I; and 3) at least one of a free radical catalyst in admixture with at least one of a living cationic catalyst; and c) curing the transparentizing composition with radiation.

An advantage of the use of the above-recited polymerizable transparentizing compositions is that the transparentized portion produced by the coating is a high quality one. Physically, the transparentized portion is strong and flexible and is highly receptive to inks and/or toner. One advantage of such good receptivity to inks and/or toner is that it allows a reverse image to be printed on the lower surface of the transparentized portion. In this manner, the reverse image is visible as a normal image through the upper surface of the transparentized portion.

Chemically, the transparentized portion of the present invention meets U.S. Postal Service specifications for reflectance and PCR. This is believed possible due to the fact that the transparentizing material penetrates the substrate substantially completely. Additionally, the resulting transparentized portion has sufficient resistance to migration and/or volatilization of the radiation cured material that it does not lose its transparency over time. While not wishing to be bound by any specific theory, this advantage is believed due to the fact that the transparentizing material is applied is 100% solids and the fact that the transparentizing material can be radiation cured almost immediately after it has been applied to the substrate since it penetrates the substrate so quickly.

Although the radiation curable transparentizing materials of the present invention penetrate the fastest when used without oligomers or prepolymers, there may be occasions when the need for specific physical and/or chemical properties in the transparentized portion outweigh the need for high speed penetration. In such circumstances, oligomers and/or prepolymers may be included in the coating. For example, it may be desirable to include one or more prepolymers in the transparentizing material if, due to the nature of the cellulosic substrate, for instance, it were necessary to adjust the refractive index of the transparentizing material in order to ensure that the cured transparentizing material has a refractive index close to that of the cellulosic substrate. The preferred prepolymers for this purpose are selected from the group consisting of styrene-maleic anhydride prepolymer, styrene-acrylic acid prepolymer, and styrene-methacrylic acid prepolymer. Similarly, it may be necessary in certain situations to have a transparentized portion with extra flexibility. In such situations, an oligomer may be included in the transparentizing material. The preferred oligomers are styrene-acrylic acid oligomers or urethane acrylate oligomers. Whether or not a prepolymer and/or oligomer is included in the transparentizing material, however, it is preferable that the trans-

parentizing material have a refractive index of about 1.5 after the transparentizing material has been cured. Further, the transparentized portion of the substrate preferably has a thickness in the range of from about 0.0005 to about 0.002 inches (i.e., about  $1.27 \times 10^{-3}$  cm to about  $5.08 \times 10^{-3}$  cm).

In addition to the foregoing, the present invention provides a method of transparentizing a predetermined portion or portions of a cellulosic substrate, preferably such that a smooth interface exists between the transparentized portion and the remainder of the substrate, and preferably such that the transparentized portion has a thickness which is no greater than the thickness of the remainder of the substrate. In some embodiments, the method comprises making a predetermined portion of the substrate thinner than the remainder of the substrate such that the predetermined portion is rendered substantially transparent, and applying a transparentizing material to the predetermined portion. In other embodiments, the method comprises heating the transparentizing material prior to application to the predetermined portion of the substrate, heating the predetermined portion of the substrate prior to application of the transparentizing material, or heating both the transparentizing material and the predetermined portion of the substrate prior to application of the transparentizing material.

As mentioned, the speed at which the above-recited transparentizing material penetrates allows transparentizing to occur in a continuous, in-line process. Such a process may be a continuous flexographic printing process, gravure, or roll-metering process, with flexographic being preferred, in which the step of applying the transparentizing material to the predetermined portion occurs in the continuous printing process. The polymerizable transparentizing compositions of the present invention have a viscosity which makes them suitable as "inks" to be applied by printing techniques. The transparentizing composition is then cured immediately thereafter as a subsequent step in the continuous process. Preferably, those steps occur at a speed of about 75 to about 1000 linear feet (i.e., about 22.86 linear meters to about 304.8 linear meters) of substrate per minute.

To provide even faster penetration of the transparentizing material into the substrate, the step of applying the transparentizing material to the predetermined portion can occur simultaneously to both the upper and lower surfaces of the predetermined portion.

In the embodiment wherein the predetermined portion of the substrate is made thinner than the remainder of the substrate, this thinning may be accomplished by removing a portion of the thickness therefrom. The removal is preferably accomplished by mechanically grinding the portion. Preferably, the predetermined portion has a thickness ranging from about 0.0005 inches to about 0.002 inches (i.e., about  $1.27 \times 10^{-3}$  cm to about  $5.08 \times 10^{-3}$  cm) following the grinding operation. Alternatively, the predetermined portion can be made thinner by compressing, such as by calendaring the predetermined portion to a predetermined thickness. Preferably, such predetermined thickness ranges from about 0.0005 inches to about 0.002 inches (i.e., about  $1.27 \times 10^{-3}$  cm to about  $5.08 \times 10^{-3}$  cm) following the compression of the predetermined portion.

Accordingly, it is a feature of the present invention to provide a cellulosic substrate which is suitable for use as a mailer or envelope and which has at least one transparentized portion. Further, these transparentizing materials may be applied without the need for solvents. Moreover, the present invention also provides a solventless transparentizing material which penetrates the mailer substrate very quickly and completely, and forms a cured polymeric trans-

parentized portion which not only possesses the aforementioned physical and chemical properties, but also exhibits an improved degree of transparency. In this manner, a very high-quality transparentized portion can be formed on cellulosic mailer substrates in a fast, continuous, in-line process, without the need for recovering a solvent. Further the present invention provides liquid polymerizable transparentizing compositions which exhibit good toner adhesion properties and are cured by radiation rather than by thermal polymerization and which cure both rapidly and completely. In addition, the liquid polymerizable transparentizing compositions of the present invention exhibit minimal odor and skin-irritating qualities. These features thus permit continuous, in-line transparentization.

#### BRIEF DESCRIPTION OF THE DRAWINGS

FIG. 1 is a front elevational view of a mailer having a transparentized portion showing addressee information;

FIG. 2 is a cross-sectional view of the cellulosic substrate after the predetermined portion has been thinned by grinding or compression;

FIG. 3 is a cross-sectional view of the cellulosic substrate after the thinned portion has been impregnated with a transparentizing material;

FIG. 4 is a cross-section view of the cellulosic substrate which has been impregnated with a transparentizing material without any thinning of the substrate;

FIG. 5 is a front-elevational view of the cellulosic substrate of FIG. 3 or FIG. 4 in which a reverse image is printed on the lower surface of the transparentized portion; and

FIG. 6 is a rear view of the lower surface of the cellulosic substrate shown in FIG. 5.

#### DETAILED DESCRIPTION OF THE INVENTION

Referring now to FIG. 1, a mailer or envelope 10 is formed from the cellulosic substrate 12 of the present invention. Substrate 12 includes a transparentized portion 14. Transparentized portion 14 allows the addressee information 16, on the inside of mailer 10, to be viewed from the outside of mailer 10. Examples of addressee information 16 on the inside of mailer 10 include 1) printing on a separate insert, 2) printing the rear inside surface of the mailer 10, or 3) printing on the rear inside surface of the transparentized portion 14. Mailer 10 can be any type of mailer or envelope. For example, mailer 10 could be an inter-office mailer or one which is mailed through the U.S. Postal Service. In addition, mailer 10 could be designed to accept a facsimile transmission sheet directly from a facsimile transmission device in order to keep information contained within the facsimile transmission sheet confidential, except for addressee information.

Referring now generally to FIGS. 2 and 3, the features of the cellulosic substrate of the present invention which utilizes a thinning of the substrate 12 will be described, where like reference numerals refer to like features. Transparentized portion 14 of substrate 12 has an upper surface 18 and a lower surface 20. When substrate 12 is used to form a mailer, upper surface 18 will be on the outside of the mailer, while lower surface 20 will be in the inside of the mailer. Transparentized portion 14 preferably has a smooth interface 22 between:

- 1) the upper surface 18 and the lower surface 20 of the transparentized portion 14 and
- 2) the remainder of substrate 12.

In this manner no loose or sharp edges are present on the substrate to get caught in printers or other process machinery.

In addition, in FIGS. 2 and 3, transparentized portion 14 has a thickness which is less than the thickness "t" of the remainder of the substrate. As a consequence, transparentized portion 14 does not increase the thickness of substrate 12. Thus, numerous ones of mailers or envelopes formed from substrate 12 can be placed into tall, stable stacks. As mentioned, such tall stacks are more convenient than short stacks and facilitate manufacturing and printing operations.

Referring now to FIG. 2, transparentized portion 14 of substrate 12 comprises an area 24 of substrate 12 which is sufficiently thinner than the remainder of the substrate 12. Area 24 can be any predetermined portion of substrate 12 whereat it is desired to place a transparentized portion.

Area 24 may be made thinner than the remainder of substrate 12 by removing a section of the thickness therefrom or by compressing it. It is preferred that transparentized portion 14 have a thickness ranging from about 0.0005 inches to about 0.002 inches (i.e., about  $1.27 \times 10^{-3}$  cm to about  $5.08 \times 10^{-3}$  cm) following the removal or of compression of the section from area 24. Although FIG. 2 shows the reduction in thickness as having been performed on the upper surface 18 of transparentized portion 14, it can also be performed to the lower surface 20, or to both surfaces. In addition, although FIG. 2 shows a reduction of the thickness of area 24 by removal of a section of the thickness therefrom or compression wherein there is a gradual sloping to area 24, one of ordinary skill in the art will readily realize that such compression or removal of thickness of area 24 may also be done such that there is a more abrupt sloping to area 24 (not shown).

In one embodiment, thinning of area 24 is accomplished by mechanically grinding away the section. A preferred means of grinding away the section of area 24 is by passing substrate 12 between a large roll and a smaller, grinding roll. Raised projections of the desired size and shape of the transparentized portion 14 are placed upon the large roll. In this manner, substrate 12 will be ground away by the grinding roll in the shape of the raised projection. Such grinding equipment is readily available commercially. An example of a suitable grinding apparatus is illustrated in U.S. Pat. No. 4,814,043 to Rausing et al., the disclosure of which is incorporated by herein by reference. It is preferred that the shape of the raised projections allow small holes to be formed in transparentized portion 14. The preferred hole size is 0.10 mm or larger.

Area 24 can also be made thinner than the remainder of substrate 12 by compressing substrate 12 at area 24 to a predetermined thickness. Preferably, such predetermined thickness ranges from about 0.0005 inches to about 0.002 inches (i.e., about  $1.27 \times 10^{-3}$  cm to about  $5.08 \times 10^{-3}$  cm) following the compression of substrate 12 at area 24. More preferably, the predetermined thickness is 0.002 inch or less (i.e.,  $5.08 \times 10^{-3}$  cm or less). The preferred technique for compressing substrate 12 at area 24 is by calendaring substrate 12, using calendaring equipment, but only at area 24. In this manner, area 24 will be thinner, and have a higher density, than the remainder of substrate 12. Compression in selected area may be accomplished by a pair of rotating cylinders, one of which has raised areas on its surface corresponding to areas to be compressed.

FIG. 4 depicts the embodiment wherein no thinning of area 24 is required to result in the transparentized portion 14 which does not increase the thickness of substrate 12. This may be accomplished by either heating area 24 by the

application of localized heat which is 50° C. to about 100° C. for about 1 to about 2 minutes prior to the application of the transparentizing material to area 24, heating the transparentizing material to a temperature of about 30° C. to about 50° C. prior to application to area 24, or heating area 24 by the application of localized heat which is 50° C. to about 100° C. for about 1 to about 2 minutes and also heating the transparentizing material to a temperature of about 30° C. to about 50° C. prior to application to heated-area 24.

As shown in FIG. 3 and FIG. 4, a portion 14 of substrate 12 is then impregnated with a radiation curable transparentizing composition of the present invention. Portion 14 can be any predetermined portion of substrate 12 where it is desired to place a transparentized portion.

The radiation curable transparentizing composition of the present invention comprises a free-radical catalyzable constituent; a cationic catalyzable constituent; and a catalyst. As used herein, the term "cationic catalyzable constituent" refers to a vinyl ether, a polyepoxide, a mixture of vinyl ethers, a mixture of polyepoxides, or a mixture of at least one of a vinyl ether and at least one of a polyepoxide. As used herein, the term "free radical catalyzable constituent" refers to compounds or Formula I or mixtures of compounds of Formula I:



wherein

R'' is any mono- or polyfunctional organic radical;  
R is H or  $CH_3$ ;  
R' is H or  $-\text{C}(\text{O})\text{C}(\text{R})=\text{CH}_2$ , with the proviso that  $-\text{C}(\text{O})\text{C}(\text{R})=\text{CH}_2$  occurs at least once;

x is an integer 0-4 and indicates the number of functional groups on R'' which are reactive with ethylene or propylene oxide;

z is an integer 1-4 and may vary independently of x and n;

n is an integer 0-20 and is independent of x and z; and wherein if any of R, R', or R'' are greater than one, their identities and the number of each may be the same or different. As used herein, the term "catalyst" refers to a photocatalyst selected from a free radical catalyst, a mixture of free radical catalysts, a living cationic catalyst, a mixture of living cationic catalysts, or mixtures of at least one of a free radical catalyst and at least one of a living cationic catalyst.

Thus, in one embodiment, there is provided a method of transparentizing a cellulosic substrate which comprises the steps of a) providing a cellulosic substrate; b) applying to at least one surface of the substrate a transparentizing composition comprising: 1) at least one of a polyepoxide; 2) and at least one of a compound or mixture of compounds of Formula I; and 3) at least one of a free radical catalyst; and c) curing the transparentizing composition with radiation.

In another embodiment, there is provided a method of transparentizing a cellulosic substrate which comprises the steps of: a) providing a cellulosic substrate; b) applying to at least one surface of the substrate a transparentizing composition comprising: 1) at least one of a vinyl ether in admixture with at least one of a polyepoxide; 2) at least one of a compound of Formula I; and 3) at least one of a free radical catalyst; and c) curing the transparentizing composition with radiation.

In another embodiment, there is provided a method of transparentizing a cellulosic substrate which comprises the

## 11

steps of: a) providing a cellulosic substrate; b) applying to at least one surface of the substrate a transparentizing composition comprising: 1) at least one of a polyepoxide; 2) at least one of a compound of Formula I; and 3) at least one of a living cationic catalyst; and c) curing the transparentizing composition with radiation.

In another embodiment, there is provided a method of transparentizing a cellulosic substrate which comprises the steps of: a) providing a cellulosic substrate; b) applying to at least one surface of the substrate a transparentizing composition comprising: 1) at least one of a vinyl ether; 2) at least one of a compound of Formula I; and 3) at least one of a living cationic catalyst; and c) curing the transparentizing composition with radiation.

In another embodiment, there is provided a method of transparentizing a cellulosic substrate which comprises the steps of: a) providing a cellulosic substrate; b) applying to at least one surface of the substrate a transparentizing composition comprising: 1) at least one of a vinyl ether in admixture with at least one of a polyepoxide; 2) at least one of a compound of Formula I; and 3) at least one of a living cationic catalyst; and c) curing the transparentizing composition with radiation.

In another embodiment, there is provided a method of transparentizing a cellulosic substrate which comprises the steps of: a) providing a cellulosic substrate; b) applying to at least one surface of the substrate a transparentizing composition comprising: 1) at least one of a polyepoxide; 2) at least one of a compound of Formula I; and 3) at least one of a free radical catalyst in admixture with at least one of a living cationic catalyst; and c) curing the transparentizing composition with radiation.

In another embodiment, there is provided a method of transparentizing a cellulosic substrate which comprises the steps of: a) providing a cellulosic substrate; b) applying to at least one surface of the substrate a transparentizing composition comprising: 1) at least one of a vinyl ether; 2) at least one of a compound of Formula I; and 3) at least one of a free radical catalyst in admixture with at least one of a living cationic catalyst; and c) curing the transparentizing composition with radiation.

In another embodiment, there is provided a method of transparentizing a cellulosic substrate which comprises the steps of: a) providing a cellulosic substrate; b) applying to at least one surface of the substrate a transparentizing composition comprising: 1) at least one of a vinyl ether in admixture with at least one of a polyepoxide; 2) at least one of a compound of Formula I; and 3) at least one of a free radical catalyst in admixture with at least one of a living cationic catalyst; and c) curing the transparentizing composition with radiation.

As stated above, the free radical catalyzable constituents for use in the present invention may be represented by Formula I:



wherein

R" is any mono- or polyfunctional organic radical;

R is H or  $\text{CH}_3$ ;

R' is H or  $-\text{C}(\text{O})\text{C}(\text{R})=\text{CH}_2$  with the proviso that  $-\text{C}(\text{O})\text{C}(\text{R})=\text{CH}_2$  occurs at least once;

x is an integer 0-4 and indicates the number of functional groups on R" which are reactive with ethylene or propylene oxide;

## 12

z is an integer 1-4 and may vary independently of x and n; n is an integer 0-20 and is independent of x and z; and wherein if any of R, R', or R" are greater than one, their identities and the number of each may be the same or different.

As used herein, the term "any organic radical" refers to any organic radical which can be attached to a hydroxyl moiety. Typical examples include mono- or multifunctional aromatic or aliphatic functionalities, wherein the aliphatic functionalities may be unsaturated, saturated, straight, branched, or cyclic in configuration.

Examples of compounds of Formula I wherein n=0 include ethylene glycol diacrylate, ethylene glycol dimethacrylate, pentaerythritol tetramethacrylate, dipentaerythritol hydroxy pentacrylate, pentacrylate, diethylene glycol dimethacrylate, 1,6-hexane diacrylate, trimethylolpropane triacrylate, and tripropylene glycol diacrylate, all of which are commercially available or readily prepared by techniques and procedures well known to one of ordinary skill in the art. For example, tripropylene glycol diacrylate is available from Sartomer or Radcure and pentacrylate is available as SR-2041 from Sartomer.

In addition, compounds of Formula I wherein n is an integer 1-20 may be prepared essentially as shown in Scheme A wherein all substituents are as previously defined unless otherwise specified.





wherein R is a straight or branched chain, saturated or unsaturated C<sub>1</sub>–C<sub>6</sub> alkyl. These cycloaliphatic polyepoxides are either commercially available or readily prepared by methods well known to those skilled in the art. For example, cycloaliphatic polyepoxide 1 is available as UVR-6110 from Union Carbide. These cycloaliphatic polyepoxides may be used in the polymerizable transparentizing composition as individual cycloaliphatic polyepoxides or as mixtures of cycloaliphatic polyepoxides. The linear cycloaliphatic diepoxides 3 are available from UCB Chemical Group, under the tradename E-CADE. The methyl hydroxy cycloaliphatic epoxide 2 is available as ETHB from UCB Chemical Group.

Suitable vinyl ethers for use in the present invention include, but are not limited to, vinyl pyrrolidone, hydroxybutyl vinyl ether, cyclohexandimethanol divinyl ether, polyester vinyl ether, fluoroalkyl vinyl ether, urethane divinyl ether, triethyleneglycol divinyl ether, vinyl/ether terminated urethane monomers and oligomers, and vinyl ether terminated ester monomers and oligomers. These vinyl ethers may be used in the polymerizable transparentizing composition as individual vinyl ethers or mixtures of vinyl ethers.

A wide variety of free-radical catalysts can be used provided they do not deleteriously affect the desired physical and chemical properties of the resultant transparentized portion. Suitable free radical catalysts for use in the present invention include, but are not limited to, xanthones, such as benzoin, ether, benzylidemethoxy ketone, acetophenones, such as 2,2 diethoxyacetophenone and t-butyl trichloroacetophenone, alkyl benzoin ethers, such as benzoin ether benzophenone, a benzophenone with an amine, such as methyl diethanolaminemethylquinoxiline, 4,4'-bis (dimethylaminebenzophenone) and chloroacetophenone. A preferred class of useful free radical photocatalysts are haloalkyl substituted aryl ketone compounds. All such photocatalysts, useful in the practice of this invention, are either readily available commercially or are easily prepared using known techniques. For example, free radical catalyst 2-hydroxy-1-[4-(hydroxy-ethoxy)phenyl]-2-methyl-1-propane is available as Iracure 2959 from Ciba Geigy. The free radical catalysts may be used in the polymerizable transparentizing composition as individual free radical catalysts or as mixtures of free radical catalysts.

Suitable living cationic catalysts for use in the present invention include may be chosen from the family of triarylsulfonium salts or the family of diaryl iodonium salts which may be expressed by the general formula III:

where III

- 1 Ar is an aromatic radical, each independently having optional substitution;

Q is a sulfur atom or iodine atom;

5 x is 3 when Q is a sulfur atom;

x is 2 when Q is an iodine atom;

y is 1 or 2; and

2 Z is  $\text{SbF}_6$  or  $\text{PF}_6^-$ .

Representative living cationic catalysts of Formula III for

10 use in the present invention include the following:

10 Representative living cationic catalysts of Formula III for use in the present invention include the following:



These living cationic catalysts are either commercially available or readily prepared by one of ordinary skill in the art. For example, a triarylsulfoniumhexafluoroantimonate salt is available as UVI 6974 from Union Carbide and a triarylsulfoniumhexafluorophosphate salt is available as UVI 6990 from Union Carbide or as CD-1011, available from Sartomer. These living cationic catalysts may be used in the

polymerizable transparentizing composition as individual living cationic catalysts or as mixtures of living cationic catalysts.

As one of ordinary skill in the art will recognize, the polyepoxide and vinyl ether constituents of the polymerizable transparentizing agents are particularly amenable to cationic catalysis whereas the acrylate and methacrylate esters of Formula I are particularly amenable to free radical catalysis. Therefore, when a dual catalyst system (i.e., both free radical and living cationic) is utilized, the polymerizable transparentizing composition may include approximately equal amounts of free radical catalyzable constituent and cationic catalyzable constituent. However, when only a free radical catalyst is utilized, for optimum results, the predominate monomer in the transparentizing composition should be the free radical catalyzable constituent. And when only a living cationic catalyst is utilized, for optimum results, the predominate monomer in the transparentizing composition should be the cationic catalyzable constituent.

Although the radiation curable transparentizing materials of the present invention penetrate the fastest when used without oligomers or prepolymers, there may be occasions when the need for specific physical and/or chemical properties in the transparentized portion outweigh the need for high speed penetration. In such circumstances, oligomers and/or prepolymers may be included in the coating. For example, it may be desirable to include one or more prepolymers in the transparentizing material if, due to the nature of the cellulosic substrate, for instance, it were necessary to adjust the refractive index of the transparentizing material in order to ensure that the cured transparentizing material has a refractive index close to that of the cellulosic substrate. The preferred prepolymers for this purpose are selected from the group consisting of styrene-maleic anhydride prepolymer, styrene-acrylic acid prepolymer, and styrene-methacrylic acid prepolymer. Similarly, it may also be necessary in certain situations to have a transparentized portion with extra flexibility. In such situations, an oligomer may be included in the polymerizable transparentizing composition as part of the free radical catalyzable reactant material. Suitable oligomers are aromatic or non-aromatic acrylates or methacrylates and include, for example, urethane acrylates, such as EBECRYL™ 6700 and EBECRYL™ 270, available from Rad-Cure, urethane methacrylates, epoxy acrylates, such as EBECRYL™ 3500 EBECRYL™ 3201, available from Rad-Cure, epoxy methacrylates, polyester acrylates, polyester methacrylates, and mixtures thereof. These oligomers are commercially available or readily prepared by techniques and procedures well known to one of ordinary skill in the art. Whether or not a prepolymer and/or oligomer is included in the transparentizing material, however, it is preferable that the transparentizing material have a refractive index of about 1.5 after the transparentizing material has been cured. Further, the transparentized portion of the substrate preferably has a thickness in the range of from about 0.0005 to about 0.002 inches (i.e., about  $1.27 \times 10^{-3}$  cm to about  $5.08 \times 10^{-3}$  cm). As used herein, the term "oligomer and/or prepolymer component" refers to an individual oligomer, an individual prepolymer, a mixture of individual oligomers, a mixture of individual prepolymers, and a mixture of at least one of an oligomer and at least one of a prepolymer.

Without oligomers or prepolymers, the radiation curable transparentization material of the present invention penetrates a cellulosic substrate quite rapidly and can be applied as a "100% solid" and still achieve a rapid rate of penetration. "100% solids" means a liquid material which can be

converted 100% to a solid upon curing (i.e., crosslinking or polymerization). Thus, it contains no residual volatiles or solvents. However, if even faster penetration is desired, a polar organic solvent can be added to the coating to lower the viscosity thereof. Preferred solvents are solvents which are polar and miscible with water and include methanol, ethanol, isopropanol, acetone and the like.

The polymerizable transparentizing composition may further include from about 0.2% to about 1% of an additive to reduce surface tension of the polymerizable liquid transparentizing material in order to increase the rate of penetration into the substrate, thus increasing production speed. These additives may be used in the polymerizable transparentizing composition as individual additives or as mixtures of additives. Suitable additives are fluorocarbons, such as FC-171 and FC-129, available from 3M or silicon prepolymers, such as SILRET 77 or DC-90, available from Union Carbide.

The radiation curable transparentizing composition of the present invention, without oligomers, prepolymers, or additives, comprises from about 10% to about 50% of a cationic catalyzable constituent; from about 40% to about 80% of a free radical catalyzable constituent; and from about 5% to about 16% of a catalyst constituent. Thus, a typical transparentizing composition of the present invention, without oligomers, prepolymers, or additives comprises 1) from about 10% to about 50% of any of a vinyl ether, polyepoxide, mixtures of vinyl ethers, mixtures of polyepoxides, or mixture of at least one of a vinyl ether and at least one of a polyepoxide; 2) from about 40% to about 80% of at least one of a compound of Formula I; and 3) from about 5 to about 16% of at least one of a free radical catalyst, at least one of a living cationic catalyst, or a mixture of at least one of a free radical catalyst and at least one of a living cationic catalyst.

Thus, according to the above, typical radiation curable transparentizing compositions, without oligomers, prepolymers, or additives, are exemplified by the following examples 1-8:

#### EXAMPLE 1

- 40 a) from about 25% to about 40% of at least one of a polyepoxide;
- 45 b) from about 40% to about 60% of at least one of a compound of Formula I; and
- 45 c) from about 5% to about 10% of at least one of a free radical catalyst.

#### EXAMPLE 2

- 50 a) from about 30% to about 35% of at least one of a polyepoxide;
- 55 b) from about 55% to about 60% of at least one of a compound of Formula I; and
- 60 c) from about 8% to about 10% of at least one of a living cationic catalyst.

#### EXAMPLE 3

- 55 a) from about 30% to about 40% of at least one of a polyepoxide;
- 60 b) from about 50% to about 60% of at least one of a compound of Formula I;
- 65 c) from about 3% to about 8% of at least one of a free radical catalyst; and
- 65 d) from about 3% to about 8% of at least one of a living cationic catalyst.

#### EXAMPLE 4

- 65 a) from about 10% to about 30% of at least one of a vinyl ether;

## 17

- b) from about 60% to about 70% of at least one of a compound of Formula I; and
- c) from about 8% to about 12% of at least one of a living cationic catalyst.

## EXAMPLE 5

- a) from about 10% to about 20% of at least one of a vinyl ether;
- b) from about 60% to about 70% of at least one of a compound of Formula I;
- c) from about 5% to about 6% of at least one of a free radical catalyst; and
- d) from about 5% to about 7% of at least one of a living cationic catalyst.

## EXAMPLE 6

- a) from about 20% to about 30% of at least one of a polyepoxide;
- b) from about 10% to about 15% of at least one of a vinyl ether;
- c) from about 40% to about 50% of at least one of a compound of Formula I; and
- d) from about 5% to about 10% of at least one of a living cationic catalyst.

## EXAMPLE 7

- a) from about 20% to about 30% of at least one of a polyepoxide;
- b) from about 10% to about 15% of at least one of a vinyl ether;
- c) from about 40% to about 50% of at least one of a compound of Formula I; and
- d) from about 8% to about 10% of at least one of a free radical catalyst.

## EXAMPLE 8

- a) from about 20% to about 30% of at least one of a polyepoxide;
- b) from about 10% to about 15% of at least one of a vinyl ether;
- c) from about 40% to about 45% of at least one of a compound of Formula I;
- d) from about 4% to about 6% of at least one of a free radical catalyst; and
- e) from about 8% to about 10% of at least one of a living cationic catalyst.

The radiation curable transparentizing composition of the present invention, without oligomers or prepolymers, but with additives, comprises from about 10% to about 50% of a cationic catalyzable constituent; from about 40% to about 80% of a free radical catalyzable constituent; from about 5% to about 13% of a catalyst constituent; and from about 0.5% to about 3% of an additive constituent. Thus, a typical transparentizing composition of the present invention, without oligomers or prepolymers, but with additives comprises 1) from about 10% to about 50% of any of a vinyl ether, polyepoxide, mixtures of vinyl ethers, mixtures of polyepoxides, or mixture of at least one of a vinyl ether and at least one of a polyepoxide; 2) from about 40% to about 80% of at least one of a compound of Formula I; 3) from about 5 to about 13% of at least one of a free radical catalyst, at least one of a living cationic catalyst, or a mixture of at

## 18

least one of a free radical catalyst and at least one of a living cationic catalyst; and 4) from about 0.5% to about 3% of an additive or mixture of additives.

Thus, according to the above, typical radiation curable 5 transparentizing compositions, without oligomers or prepolymers, but with an additive are exemplified by the following examples 9-16:

## EXAMPLE 9

- a) from about 25% to about 35% of at least one of a polyepoxide;
- b) from about 50% to about 70% of at least one of a compound of Formula I;
- c) from about 5% to about 10% of at least one of a free radical catalyst; and
- d) from about 1 to about 3% of an additive or mixture of additives.

## EXAMPLE 10

- a) from about 30% to about 35% of at least one of a polyepoxide;
- b) from about 50% to about 55% of at least one of a compound of Formula I;
- c) from about 8% to about 10% of at least one of a living cationic catalyst; and
- d) from about 1% to about 2% of an additive or mixture of additives.

## EXAMPLE 11

- a) from about 25% to about 40% of at least one of a polyepoxide;
- b) from about 40% to about 60% of at least one of a compound of Formula I;
- c) from about 2% to about 5% of at least one of a free radical catalyst;
- d) from about 4% to about 6% of at least one of a living cationic catalyst; and
- e) from about 1% to about 2% of an additive or mixture of additives.

## EXAMPLE 12

- a) from about 10% to about 20% of at least one of a vinyl ether;
- b) from about 60% to about 70% of at least one of a compound of Formula I;
- c) from about 8% to about 10% of at least one of a living cationic catalyst; and
- d) from about 1% to about 2% of an additive or mixture of additives.

## EXAMPLE 13

- a) from about 10% to about 20% of at least one of a vinyl ether;
- b) from about 60% to about 70% of at least one of a compound of Formula I;
- c) from about 5% to about 6% of a free radical catalyst;
- d) from about 5% to about 7% of at least one of a living cationic catalyst; and
- e) from about 1% to about 2% of an additive or mixture of additives.

## EXAMPLE 14

- a) from about 20% to about 30% of at least one of a polyepoxide;

**19**

- b) from about 10% to about 15% of at least one of a vinyl ether;
- c) from about 40% to about 50% of at least one of a compound of Formula I;
- d) from about 5% to about 10% of at least one of a living cationic catalyst; and
- e) from about 0.5% to about 1% of an additive or mixture of additives.

**EXAMPLE 15**

- a) from about 20% to about 30% of at least one of a polyepoxide;
- b) from about 10% to about 15% of at least one of a vinyl ether;
- c) from about 40% to about 50% of at least one of a compound of Formula I;
- d) from about 5% to about 10% of at least one of a free radical catalyst; and
- e) from about 0.5% to about 1% of an additive or mixture of additives.

**EXAMPLE 16**

- a) from about 20% to about 30% of at least one of a polyepoxide;
- b) from about 10% to about 15% of at least one of a vinyl ether;
- c) from about 40% to about 45% of at least one of a compound of Formula I;
- d) from about 3% to about 5% of at least one of a free radical catalyst;
- e) from about 6% to about 8% of at least one of a living cationic catalyst; and
- f) from about 0.5% to about 1% of an additive or mixture of additives.

The radiation curable transparentizing composition of the present invention, with oligomers and/or prepolymers, but without additives, comprises from about 10% to about 50% of a cationic catalyzable constituent; from about 40% to about 80% of a free radical catalyzable constituent; from about 5% to about 13% of a catalyst constituent; and from about 2% to about 50%, preferably from about 2% to about 12% of an oligomer and/or prepolymer component. Thus, a typical transparentizing composition of the present invention, with oligomers and/or prepolymers, but without additives comprises 1) from about 10% to about 50% of any of a vinyl ether, polyepoxide, mixtures of vinyl ethers, mixtures of polyepoxides, or mixture of at least one of a vinyl ether and at least one of a polyepoxide; 2) from about 40% to about 80% of at least one of a compound of Formula I; 3) from about 5 to about 13% of at least one of a free radical catalysts, at least one of a living cationic catalyst, or a mixture of at least one of a free radical catalyst and at least one of a living cationic catalyst; and 4) from about 2% to about 50%, preferably from about 2% to about 12% of an oligomer and/or prepolymer component.

Thus, according to the above, typical radiation curable transparentizing compositions, with oligomers, prepolymers, but without an additive component are exemplified by the following examples 17-24:

**EXAMPLE 17**

- a) from about 25% to about 35% of at least one of a polyepoxide;

**20**

- b) from about 50% to about 70% of at least one of a compound of Formula I;
- c) from about 4% to about 6% of at least one of a free radical catalyst; and
- d) from about 3 to about 6% of an oligomer and/or prepolymer component.

**EXAMPLE 18**

- 10 a) from about 30% to about 35% of at least one of a polyepoxide;
- b) from about 50% to about 55% of at least one of a compound of Formula I;
- c) from about 5% to about 10% of at least one of a living cationic catalyst; and
- d) from about 5% to about 8% of an oligomer and/or prepolymer component.

**EXAMPLE 19**

- 20 a) from about 30% to about 40% of at least one of a polyepoxide;
- b) from about 50% to about 60% of at least one of a compound of Formula I;
- c) from about 3% to about 4% of at least one of a free radical catalyst;
- d) from about 4% to about 6% of at least one of a living cationic catalyst; and
- e) from about 3% to about 4% of an oligomer and/or prepolymer component.

**EXAMPLE 20**

- 25 a) from about 12% to about 20% of at least one of a vinyl ether;
- b) from about 60% to about 70% of at least one of a compound of Formula I;
- c) from about 8% to about 10% of at least one of a living cationic catalyst; and
- 30 d) from about 5% to about 10% of an oligomer and/or prepolymer component.

**EXAMPLE 21**

- 45 a) from about 10% to about 20% of at least one of a vinyl ether;
- b) from about 60% to about 70% of at least one of a compound of Formula I;
- c) from about 5% to about 6% of at least one of a free radical catalyst;
- d) from about 5% to about 7% of at least one of a living cationic catalyst; and
- e) from about 4% to about 5% of an oligomer and/or prepolymer component.

**EXAMPLE 22**

- 55 a) from about 20% to about 30% of at least one of a polyepoxide;
- b) from about 10% to about 15% of at least one of a vinyl ether;
- c) from about 40% to about 45% of at least one of a compound of Formula I;
- d) from about 5% to about 10% of at least one of a living cationic catalyst; and
- e) from about 4% to about 5% of an oligomer and/or prepolymer component.

**21****EXAMPLE 23**

- a) from about 20% to about 30% of at least one of a polyepoxide;
- b) from about 10% to about 15% of at least one of a vinyl ether;
- c) from about 40% to about 45% of at least one of a compound of Formula I;
- d) from about 8% to about 10% of at least one of a free radical catalyst; and
- e) from about 4% to about 5% of an oligomer and/or prepolymer component.

**EXAMPLE 24**

- a) from about 20% to about 30% of at least one of a polyepoxide;
- b) from about 10% to about 15% of at least one of a vinyl ether;
- c) from about 40% to about 45% of at least one of a compound of Formula I;
- d) from about 3% to about 5% of at least one of a free radical catalyst;
- e) from about 6% to about 8% of at least one of a living cationic catalyst; and
- f) from about 3% to about 5% of an oligomer and/or prepolymer component.

The radiation curable transparentizing composition of the present invention, with oligomers and/or prepolymers, and with additives, comprises from about 10% to about 50% of a cationic catalyzable constituent; from about 30% to about 80% of a free radical catalyzable constituent; from about 5% to about 13% of a catalyst constituent; from about 1% to about 50%, preferably from about 1% to about 10% of an oligomer and/or prepolymer component; and from about 0.2% to about 2% of an additive. Thus, a typical transparentizing composition of the present invention, with oligomers and/or prepolymers, and with additives comprises 1) from about 10% to about 50% of any of a vinyl ether, polyepoxide, mixtures of vinyl ethers, mixtures of polyepoxides, or mixture of at least one of a vinyl ether and at least one of a polyepoxide; 2) from about 30% to about 80% of at least one of a compound of Formula I; 3) from about 5% to about 13% of at least one of a free radical catalyst, at least one of a living cationic catalyst, or a mixture of at least one of a free radical catalyst and at least one of a living cationic catalyst; 4) from about 1% to about 50%, preferably from about 1% to about 10% of an oligomer and/or prepolymer component; and 5) from about 0.2% to about 2% of an additive or mixture of additives.

Thus, according to the above, typical radiation curable transparentizing compositions, with oligomers and/or prepolymers and with an additive component are exemplified by the following examples 25-32:

**EXAMPLE 25**

- a) from about 25% to about 35% of at least one of a polyepoxide;
- b) from about 50% to about 70% of at least one of a compound of Formula I;
- c) from about 4% to about 6% of at least one of a free radical catalyst;
- d) from about 3 to about 5% of an oligomer and/or prepolymer component; and
- e) from about 0.5% to about 2% of an additive or mixture of additives.

**22****EXAMPLE 26**

- a) from about 30% to about 35% of at least one of a polyepoxide;
- b) from about 50% to about 55% of at least one of a compound of Formula I;
- c) from about 5% to about 10% of at least one of a living cationic catalyst;
- d) from about 5% to about 8% of an oligomer and/or prepolymer component; and
- e) from about 1% to about 2% of an additive or mixture of additives.

**EXAMPLE 27**

- a) from about 10% to about 30% of at least one of a polyepoxide;
- b) from about 30% to about 60% of at least one of a compound of Formula I;
- c) from about 3% to about 6% of at least one of a free radical catalyst;
- d) from about 2% to about 6% of at least one of a living cationic catalyst;
- e) from about 1% to about 10% of an oligomer and/or prepolymer component; and
- f) from about 0.2% to about 1% of an additive or mixture of additives.

**EXAMPLE 28**

- a) from about 10% to about 20% of at least one of a vinyl ether;
- b) from about 60% to about 70% of at least one of a compound of Formula I;
- c) from about 8% to about 10% of at least one of a living cationic catalyst;
- d) from about 5% to about 10% of an oligomer and/or prepolymer component; and
- e) from about 1% to about 2% of an additive or mixture of additives.

**EXAMPLE 29**

- a) from about 10% to about 20% of at least one of a vinyl ether;
- b) from about 60% to about 70% of at least one of a compound of Formula I;
- c) from about 5% to about 6% of at least one of a free radical catalyst;
- d) from about 5% to about 7% of at least one of a living cationic catalyst;
- e) from about 4% to about 5% of an oligomer and/or prepolymer component; and
- f) from about 1% to about 2% of an additive or mixture of additives.

**EXAMPLE 30**

- a) from about 20% to about 30% of at least one of a polyepoxide;
- b) from about 10% to about 15% of at least one of a vinyl ether;
- c) from about 40% to about 45% of at least one of a compound of Formula I;
- d) from about 5% to about 10% of at least one of a living cationic catalyst;

23

e) from about 4% to about 6% of an oligomer and/or prepolymer component; and

f) from about 0.5% to about 1% of an additive or mixture of additives.

## EXAMPLE 31

a) from about 20% to about 30% of at least one of a 10 polyepoxide;

b) from about 10% to about 15% of at least one of a vinyl ether;

c) from about 40% to about 45% of at least one of a 15 compound of Formula I;

d) from about 5% to about 10% of at least one of a free radical catalyst;

e) from about 4% to about 6% of an oligomer and/or 20 prepolymer component; and

f) from about 0.5% to about 1% of an additive or mixture of additives.

## EXAMPLE 32

a) from about 20% to about 30% of at least one of a polyepoxide;

b) from about 10% to about 15% of at least one of a vinyl ether;

c) from about 40% to about 45% of at least one of a 30 compound of Formula I;

d) from about 3% to about 5% of at least one of a free radical catalyst;

e) from about 6% to about 8% of at least one of a living 40 cationic catalyst;

f) from about 3% to about 5% of an oligomer and/or prepolymer component; and

g) from about 0.5% to about 1% of an additive or mixture 45 of additives.

A preferred radiation-curable transparentizing composition of the present invention comprises:

a) from about 30% to about 40% of a polyepoxide of the 50 formula



b) from about 50% to about 60% of tripropyleneglycol 60 diacrylate;

c) from about 3% to about 6% of pentacrylate;

d) about 4.5% of 2-hydroxy-1-[4-(hydroxy-ethoxy) 65 phenyl]-2-methyl-1-propane; and

e) about 5.5% of a triarylsulfonium hexafluorophosphate salt of the formula

24



A more preferred radiation-curable transparentizing composition of the present invention comprises:

a) from about 30% to about 32% of a polyepoxide of the formula



b) from about 52% to about 55% of tripropyleneglycol 30 diacrylate;

c) from about 4% to about 5% of pentacrylate;

d) about 4.5% of 2-hydroxy-1-[4-(hydroxy-ethoxy) 35 phenyl]-2-methyl-1-propane; and

e) about 5.5% of a triarylsulfonium hexafluorophosphate salt of the formula



A still more preferred radiation-curable transparentizing composition of the present invention comprises:

a) about 31.5% of a polyepoxide of the formula



b) about 54% of tripropyleneglycol diacrylate;

c) about 4.5% of pentacrylate;

d) about 4.5% of 2-hydroxy-1-[4-(hydroxy-ethoxy) 65 phenyl]-2-methyl-1-propane; and

e) about 5.5% of a triarylsulfonium hexafluorophosphate salt of the formula



Yet a still more preferred radiation-curable transparentizing composition of the present invention comprises:

a) about 31.5% of a polyepoxide of the formula



b) about 54% of tripropyleneglycol diacrylate;

c) about 4.5% of pentacrylate;

d) about 4.5% of 2-hydroxy-1-[4-(hydroxy-ethoxy)phenyl]-2-methyl-1-propane; and

e) about 5.5% of a triarylsulfonium hexafluorophosphate salt of the formula



Preferably, the polymerizable transparentizing composition is cured by exposure to one of radiation—either electron beam, visible or ultraviolet radiation. Curing causes the polymerizable constituents of the transparentizing material to polymerize, thus making a permanently transparentized portion. Once the transparentizing composition is cured, it is a solid and will not migrate or volatilize. Advantageously, the rapidity with which the present transparentizing material penetrates the substrate allows curing thereof almost immediately following its application to the substrate, thus providing substantially no opportunity for the material to migrate or volatilize beyond the area to which it has been applied. The liquid polymerizable transparentizing compositions of the present invention are cured rapidly and completely. For example, transparentizing compositions of the present invention which contain both free radical and living cationic catalysts will typically demonstrate a 95% or greater completion of cross-linking reactions. In addition, compositions containing living cationic catalysts, either alone or in combination with free radical catalysts, will continue to cure to some extent even after exposure to radiation has ceased. And while the application of radiation alone activates both the free radical and living cationic catalysts components of the polymerizable transparentizing

composition to initiate cross-linking, the crosslinking rate may be enhanced by the application of heat which may be conveniently provided by infrared radiation. Heat is particularly effective in promoting the activity of the cationic catalyst.

The speed at which the transparentizing material of the present invention penetrates substrate 12 allows transparentizing to occur in a continuous, in-line process. Such a process can include any conventional printing method such as flexographic, gravure, or screen. A continuous transparentization process can be set up in which the transparentizing material is first applied to area 24 in a flexographic printing press and then cured immediately thereafter by electron beam, visible, or ultraviolet radiation.

15 In the case of a flexographic printing press in combination with ultraviolet curing, for example, an acceptable rate of transparentization (i.e., applying the transparentizing material to substrate 12 and curing it) is from about 75 to about 150 linear feet (i.e., about 22.9 meters to about 45.72 meters) of substrate per minute. Obviously faster production speeds are usually preferred. One expedient for increasing production speed is to mildly heat the substrate and/or transparentizing material (50° C.–100° C.) to effectively reduce viscosity and increase the penetration rate. The preferred viscosity of the coating at 25° C. is from about 30 to about 100 centipoise and more preferably from about 30 to about 70 centipoise. The preferred wavelength of the ultraviolet curing light is from about 200 to about 400 nanometers, and the preferred ultraviolet curing light capacity is from about 300 to about 600 watts per inch of substrate width.

20 The transparentizing material can be applied to one or both sides of substrate 12 at area 24. It is preferred, however, that it be applied simultaneously to both sides of area 24. Such simultaneous application provides even faster penetration of the transparentizing material into the substrate.

25 Advantageously, the use of polymerizable transparentizing composition of the present invention, without oligomers or prepolymers, results in a transparentizing material which not only penetrates substrate 12 quickly, but also produces 30 a transparentized portion 14 which meets all of the desired physical and chemical properties. Physically, transparentized portion 14 is strong, flexible and durable such that it will maintain its transparency when subjected to rough handling. In addition, transparentized portion 14 is highly 35 receptive to inks and/or toners. An advantage of such good receptivity to inks and/or toners is that it allows a reverse image to be printed on the lower surface of the transparentized portion. This feature will be explained in greater detail below.

40 Chemically, the transparentized portion 14 has sufficient 45 resistance to ultraviolet radiation that it does not lose its transparency over time. The transparentized portion meets U.S. Postal Service specifications for reflectance and PCR. This is believed possible due to the fact that the above-recited monomers achieve substantially complete penetration of substrate 12. Additionally, transparentized portion 14 has sufficient resistance to migration and/or volatilization of the radiation cured transparentizing material that it does not lose its transparency over time. Due to the rapid penetration 50 of the transparentizing material into substrate 12, the transparentizing material can be cured almost immediately after it has been applied to area 24. Moreover, although compatible with polar organic solvents, the transparentizing material of the present invention does not require the use of 55 organic solvents. Therefore, it is less volatile after curing than one containing an organic solvent, thus further reducing the tendency to migrate or volatilize.

It is preferred that the transparentizing material, once cured, have a refractive index as close as possible to that of substrate **12**. This will ensure that the transparentized portion **14** will be sufficiently transparent. Most cellulosic substrates have a refractive index of around 1.5. Thus, the preferred refractive index of the cured coating is similarly around 1.5.

However, some cellulosic substrates have a refractive index which is greater than 1.5. With such substrates, it may be desirable to include one or more prepolymers with the transparentizing material in order to increase the refractive index of the cured transparentizing material to substantially match that of the substrate. Typically, 1.55 is the highest value that the refractive index of the cured transparentizing material will need to attain in this manner. The preferred prepolymers for this function include styrene-maleic anhydride, styrene-acrylic acid and, styrene-methacrylic acid. The most preferred prepolymer of this group is styrene-maleic anhydride.

It may also be desirable in certain situations to have a transparentized portion with extra flexibility. For this purpose, an oligomer may be included with the transparentizing material. The preferred oligomers in this instance are urethane acrylate oligomer and styrene-acrylic oligomer.

Referring now to FIGS. 5 and 6, the reverse image printing feature of the present invention will be discussed. FIG. 6 is a view of the lower surface **30** of substrate **12** and shows reverse image **80**, which has been printed on the lower surface **20** of transparentized portion **14**. Reverse image **80** can be printed with any conventional printing means, such as laser printing, ion deposition printing, ink jet printing, or thermal transfer techniques. FIG. 5 is a view from the upper surface **82** of substrate **12** and shows reverse image **80** as it appears through the upper surface **18** of transparentized portion **14**—i.e., as a normal image. When substrate **12** is used to form a mailer, the normal image of reverse image **80** is the image that will be seen by the observer.

While representative embodiments and certain details have been shown for purposes of illustrating the invention, it will be apparent to those skilled in the art that various changes in the methods and apparatus disclosed herein may be made without departing from the scope of the invention, which is defined in the appended claims.

What is claimed is:

1. A method of transparentizing a cellulosic substrate which comprises the steps of:
  - a) providing a cellulosic substrate;
  - b) applying to at least one surface of the substrate a transparentizing composition comprising:
    - i) a cationic catalyzable constituent selected from a vinyl ether, 2) a polyepoxide, 3) a mixture of vinyl ethers, 4) a mixture of polyepoxides, or 5) a mixture of at least one of a vinyl ether and at least one of a polyepoxide;
    - ii) a free radical catalyzable constituent selected from at least one compound of the Formula I:



wherein,

$R''$  is any mono- or polyfunctional organic radical;  
 $R$  is H or  $CH_3$ ;

$R'$  is H or  $-C(O)C(R)=CH_2$ , with the proviso that  $-C(O)C(R)=CH_2$  occurs at least once;  
 $x$  is an integer 0-4 and indicates the number of functional groups on  $R''$  which are reactive with ethylene or propylene oxide;  
 $z$  is an integer 1-4 and may vary independently of  $x$  and  $n$ ;  
 $n$  is an integer 0-20 and is independent of  $x$  and  $z$ ;

10 wherein if any of  $R$ ,  $R'$ , or  $R''$  are greater than one, their identities and the number of each may be the same or different;

ii) a catalyst constituent comprising at least one free radical catalyst and at least one living cationic catalyst; and

c) curing the transparentizing composition with radiation.

2. A method according to claim 1 wherein the polyepoxide is selected from



wherein  $R$  is a straight or branched chain, saturated or unsaturated  $C_1-C_6$  alkylene.

3. A method according to claim 1 wherein the vinyl ether is selected from vinyl pyrrolidone, hydroxybutyl vinyl ether, cyclohexandimethanol divinyl ether, polyester vinyl ether, fluoroalkyl vinyl ether, urethane divinyl ether, triethyleneglycol divinyl ether, vinyl/ether terminated urethane monomers and oligomers, or vinyl ether terminated ester monomers and oligomers.

4. A method according to claim 1 wherein the free radical catalyst is selected from 2-hydroxy-1-[4-(hydroxy-ethoxy)phenyl]-2-methyl-1-propane, benzoin ether benzophenone, methyl diethanolaminemethylquinoxiline 4,4'-bis(dimethylaminebenzophenone, 2,2-diethoxyacetophenone, or t-butyltrichloroacetophenone.

5. A method according to claim 1 wherein the living cationic catalyst is a triarylsulfonium salt or a diaryl iodonium salt of the formula:



where

11  $Ar$  is an aromatic radical, each independently having optional substitution;

$Q$  is a sulfur atom or iodine atom;

$x$  is 3 when  $Q$  is a sulfur atom;

$x$  is 2 when  $Q$  is an iodine atom;

$y$  is 1 or 2; and

$Z$  is  $SbF_6$  or  $PF_6$ .

29

6. A method according to claim 5 wherein the living cationic catalyst is selected from:



7. A method according to claim 1 wherein the transparentizing composition further includes an oligomer, a prepolymer, or mixtures thereof.

8. The method of claim 7 wherein the prepolymer is selected from the group styrene-maleic anhydride prepolymer, styrene-acrylic acid prepolymer, or styrene-methacrylic acid prepolymer.

9. The method of claim 7 wherein the oligomer is selected from styrene-acrylic acid oligomer or urethane acrylate oligomer.

10. A method according to claim 1 wherein the transparentizing composition further includes an additive or mixture of additives.

11. A method according to claim 10 wherein the additive is a fluorocarbon or a silicon prepolymer.

30

12. A method according to claim 10 wherein the transparentizing composition further includes an oligomer, prepolymer, or mixtures thereof.

13. A method according to claim 1 wherein the cationic catalyzable constituent comprises at least one of a polyepoxide.

14. A method according to claim 1 wherein the cationic catalyzable constituent comprises at least one of a vinyl ether in admixture with at least one of a polyepoxide.

15. A method according to claim 1 wherein the cationic catalyzable constituent comprises at least one of a vinyl ether.

16. A method according to claim 1 wherein the transparentizing composition comprises:

a) from about 30% to about 40% of at least one of a polyepoxide;

b) from about 50% to about 60% of at least one of a compound of Formula I;

c) from about 3% to about 8% of at least one of a free radical catalyst; and

d) from about 3% to about 8% of at least one of a living cationic catalyst.

17. A method according to claim 16 wherein the radiation-curable transparentizing composition of the present invention comprises:

a) from about 30% to about 40% of a polyepoxide of the formula



b) from about 50% to about 60% of tripropyleneglycol diacrylate;

c) from about 3% to about 6% of pentacrylate;

d) about 4.5% of 2-hydroxy-1-[4-(hydroxy-ethoxy)phenyl]-2-methyl-1-propane; and

e) about 5.5% of a triarylsulfonium hexafluorophosphate salt of the formula



18. A method according to claim 17 wherein the radiation-curable transparentizing composition of the present invention comprises:

a) from about 30% to about 32% of a polyepoxide of the formula

31



- b) from about 52% to about 55% of tripropylene glycol diacrylate;  
 c) from about 4% to about 5% of pentacrylate;  
 d) about 4.5% of 2-hydroxy-1-[4-(hydroxy-ethoxy) phenyl]-2-methyl-1-propane; and  
 e) about 5.5% of a triarylsulfonium hexafluorophosphate salt of the formula



19. A method according to claim 18 wherein the radiation-curable transparentizing composition of the present invention comprises:

- a) about 31.5% of a polyepoxide of the formula



- b) about 54% of tripropylene glycol diacrylate;  
 c) about 4.5% of pentacrylate;  
 d) about 4.5% of 2-hydroxy-1-[4-(hydroxy-ethoxy) phenyl]-2-methyl-1-propane; and  
 e) about 5.5% of a triarylsulfonium hexafluorophosphate salt of the formula



20. A method according to claim 1 wherein the composition is applied to the substrate as a 100% solids liquid.

21. A method according to claim 1 wherein the composition has a refractive index of about 1.5 when cured.

22. A cellulosic substrate having at least one transparentized portion, said transparentized portion comprising an area of said substrate which has been impregnated with a polymerizable transparentizing material comprising:

32

- i) a cationic catalyzable constituent selected from a vinyl ether, 2) a polyepoxide, 3) a mixture of vinyl ethers, 4) a mixture of polyepoxides, or 5) a mixture of at least one of a vinyl ether and at least one of a polyepoxide;  
 ii) a free radical catalyzable constituent selected from at least one compound of the Formula I:



15 wherein,

R'' is any mono- or polyfunctional organic radical;  
 R is H or CH<sub>3</sub>;

R' is H or  $-\text{C}(\text{O})\text{C}(\text{R})=\text{CH}_2$ , with the proviso that  $-\text{C}(\text{O})\text{C}(\text{R})=\text{CH}_2$  occurs at least once;

x is an integer 0-4 and indicates the number of functional groups on R'' which are reactive with ethylene or propylene oxide;

z is an integer 1-4 and may vary independently of x and n;

n is an integer 0-20 and is independent of x and z; and wherein if any of R, R', or R'' are greater than one, their identities and the number of each may be the same or different;

- iii) a catalyst constituent comprising at least one free radical catalyst and at least one living cationic catalyst; wherein the transparentizing composition has been cured with radiation.

23. A cellulosic substrate according to claim 22 wherein the transparentizing composition comprises:

- a) from about 30% to about 40% of at least one of a polyepoxide;  
 b) from about 50% to about 60% of at least one of a compound of Formula I;  
 c) from about 3% to about 8% of at least one of a free radical catalyst; and  
 d) from about 3% to about 8% of at least one of a living cationic catalyst.

24. A cellulosic substrate according to claim 23 wherein the transparentizing composition comprises:

- a) from about 30% to about 40% of a polyepoxide of the formula



- b) from about 50% to about 60% of tripropylene glycol diacrylate;  
 c) from about 3% to about 6% of pentacrylate;  
 d) about 4.5% of 2-hydroxy-1-[4-(hydroxy-ethoxy) phenyl]-2-methyl-1-propane; and  
 e) about 5.5% of a triarylsulfonium hexafluorophosphate salt of the formula

33



25. A cellulosic substrate according to claim 24 wherein the radiation-curable transparentizing composition of the present invention comprises:

a) from about 30% to about 32% of a polyepoxide of the formula



b) from about 52% to about 55% of tripropyleneglycol diacrylate;

c) from about 4% to about 5% of pentaacrylate;

d) about 4.5% of 2-hydroxy-1-[4-(hydroxy-ethoxy) phenyl]-2-methyl-1-propane; and

e) about 5.5% of a triarylsulfonium hexafluorophosphate salt of the formula



26. A cellulosic substrate according to claim 25 wherein the radiation-curable transparentizing composition of the present invention comprises:

a) about 31.5% of a polyepoxide of the formula



b) about 54% of tripropyleneglycol diacrylate;

c) about 4.5% of pentaacrylate;

d) about 4.5% of 2-hydroxy- 1-[4-(hydroxy-ethoxy) phenyl]-2-methyl- 1-propane; and

e) about 5.5% of a triarylsulfonium hexafluorophosphate salt of the formula

5  
10

34



27. A cellulosic substrate according to claim 26 wherein the transparentizing composition comprises:

a) about 31.5% of a polyepoxide of the formula



b) about 54% of tripropyleneglycol diacrylate;

c) about 4.5% of pentaacrylate;

d) about 4.5% of 2-hydroxy-1-[4-(hydroxy-ethoxy) phenyl]-2-methyl-1-propane; and

e) about 5.5% of a triarylsulfonium hexafluorophosphate salt of the formula:

20  
25  
30  
35



40  
45

28. The substrate of claim 22 wherein the transparentized portion has a thickness in the range of from about 0.0005 to about 0.002 inches.

29. The substrate of claim 22 wherein the substrate is in the form of an envelope or mailer having at least a first ply and a second ply, with the transparentized portion on the first ply.

30. A method of transparentizing a cellulosic substrate which comprises the steps of:

a) providing a cellulosic substrate;

b) applying to at least one surface of the substrate a transparentizing composition comprising:

i) a cationic catalyzable constituent selected from a vinyl ether, 2) a polyepoxide, 3) a mixture of vinyl ethers, 4) a mixture of polyepoxides, or 5) a mixture of at least one of a vinyl ether and at least one of a polyepoxide;

ii) a free radical catalyzable constituent selected from at least one compound of the Formula I:

50  
55  
60

35



wherein,

R" is any mono- or polyfunctional organic radical;

R is H or  $\text{CH}_3$ ;

$R'$  is H or  $-\text{C}(\text{O})\text{C}(\text{R})=\text{CH}_2$ , with the proviso that  $-\text{C}(\text{O})\text{C}(\text{R})=\text{CH}_2$  occurs at least once;

x is an integer 0-4 and indicates the number of functional groups on R" which are reactive with ethylene or propylene oxide;

$z$  is an integer 1–4 and may vary independently of  $x$  and  $n$ ;

36

n is an integer 0–20 and is independent of x and z;  
and

wherein if any of  $R$ ,  $R'$ , or  $R''$  are greater than one, their identities and the number of each may be the same or different;

iii) a catalyst constituent comprising at least one living cationic catalyst; and

c) curing the transparentizing composition with radiation.

31. A method according to claim 30 wherein the cationic  
10 catalyzable constituent comprises at least one of a polyep-  
oxide.

**32.** A method according to claim 30 wherein the cationic catalyzable constituent comprises at least one of a vinyl ether in admixture with at least one of a polyepoxide.

\* \* \* \*